

Sept. 29, 1931.

W. C. BENNETT

1,825,625

STIFFENING MEMBER FOR BOOTS AND SHOES

Filed June 15, 1923



*Fig. 3.*



*Inventor.*

Wallace C. Bennett  
by Jas. H. Schuehill  
Atty.

## UNITED STATES PATENT OFFICE

WALLACE C. BENNETT, OF HINGHAM, MASSACHUSETTS, ASSIGNOR TO BENNETT BOX CO., OF BOSTON, MASSACHUSETTS, A CORPORATION OF MASSACHUSETTS

## STIFFENING MEMBER FOR BOOTS AND SHOES

Application filed June 15, 1923. Serial No. 645,520.

This invention relates to a stiffening member for a boot or shoe, and particularly to a box toe, counter and shank therefor.

The object of the invention is, in general to provide a novel, durable and superior stiffening member for a boot or shoe which may be economically manufactured and incorporated into the boot or shoe with a minimum effort and at minimum expense.

To this end, the improved stiffening member comprises a composite material made up of a supporting fabric, preferably of canvas, cloth, screening or other foraminous material; an absorbent mass of loosely-matted fibres derived from wood, as by a pulping process; and a dense, continuous body of dried and/or hardened saturant. The latter, which serves, and is hereinafter referred to, as the stiffening composition, may and preferably will include a material such as rubber latex which is capable of imparting sufficient flexibility to the composition when dried to prevent cracking of the finished stiffening member and to render the latter resiliently flexible when the boot or shoe is worn.

In practice, the stiffening composition may and preferably will be applied to both the wood pulp and the reinforcing fabric and then permitted to dry with such layers superposed one upon the other to form a composite sheet from which blanks of the requisite shape may be cut or dried out. In the use of such blanks, the operator at the lasting machine may and preferably will dip the blanks into the stiffening composition, and then incorporate them while in a flexible condition into the boots or shoes during the lasting operation, in which the top or central portion of the box toe is rendered relatively resiliently flexible and the side walls thereof relatively stiff and non-flexible.

These and other features of the invention will be hereinafter described and particularly pointed out in the claims at the end of this specification.

In the drawings, Fig. 1 represents a shoe in side elevation embodying the present stiffening member;

Fig. 2 is a cross-section through the toe portion of the shoe;

Fig. 3 is a plan of the stiffener blank used in the production of a box toe, with portions broken away;

Fig. 4 is a section on line 4—4 of Fig. 3; and

Fig. 5 is a plan with portions broken away 55 of a counter blank embodying the present invention.

Referring to the drawings, 10 represents a blank of fibrous material preferably composed of two layers 11, 12, one of wood pulp 60 and the other of cloth, canvas or the like, and the wood pulp layer has incorporated with it a stiffening composition 13, preferably a fluid containing concentrated sodium silicate and rubber latex.

In producing the blank 10 of fibrous material I preferably form the blank 11 from a layer or sheet of loosely-matted wood pulp, and the cloth blank 12 from a sheet of canvas or other fabric. After the blanks 11, 12 have 70 thus been formed, both are preferably immersed in the fluid stiffening composition to be saturated therewith, then withdrawn and the wood pulp blank 11 superimposed upon the cloth blank 12 and the fluid stiffening 75 composition permitted to dry and form the composite blank 10.

The basic material which I preferably employ in the stiffening composition is a soluble silicate such as sodium silicate, and in order to impart flexibility to the stiffening composition after the stiffening member has been incorporated into the shoe and dried, so as to prevent cracking thereof when the shoe is worn, I utilize a material capable of imparting 80 flexibility to the silicate, and preferably rubber latex in the fluid condition in which it may be purchased in the market. Excellent results have been obtained with a stiffening composition consisting of 75% by volume of concentrated sodium silicate solution, and 25% by volume of rubber latex.

The dried composite blanks 10 produced as above stated may be softened by immersion 95 in some of the fluid stiffening material itself by the operator at the lasting machine, and when the blanks have become sufficiently flexible, they may be withdrawn from such solution, and immediately applied to the last 100

and the lasting operation performed in the usual manner.

The loosely-matted wood pulp of which the blank 11 is composed, is not only inexpensive, but also has remarkable affinity for fluids and is capable of absorbing a maximum amount of the stiffening material. In this manner maximum strength and body is imparted to the finished stiffening member. 10 The use of concentrated or heavy silicate adds to the water resistant properties of the finished or dried stiffening member, and for this reason it is preferred to employ it instead of dilute silicate solutions. For the reason 15 that absorbent wood pulp was invented by Willis A. Boughton and is disclosed in his applications Serial No. 641,767, filed May 26, 1923, and Serial No. 283,946, filed June 8, 1928, I make no claim thereto, but rather 20 to the novel combination of a fibrous material supported by means of a fabric which, together with said fibrous material, is thoroughly impregnated with a saturant.

In the wiping operation of lasting the toe 25 portion of the shoe some of the silicate is caused to flow from the center to the sides of the blank with the result that the central or top portion of the box is rendered relatively flexible, while the sides of the box are 30 rendered relatively stiff and effectively serve to retain the shape of the box toe as the shoe is worn.

When the stiffening member comprises a counter, the blanks 11, 12 are cut into the 35 shape illustrated in Fig. 5, and the composite blank 10 formed as above stated is incorporated into the shoe in the usual manner.

It will be observed that in the preferred 40 form of the invention all of the ingredients of the stiffening material are of a colorless or milky white nature, a feature which particularly enables the stiffening member to be employed in connection with white canvas or fabric shoes without liability of soiling the 45 latter. The present stiffening member may be made relatively light in weight, thus rendering its use particularly advantageous in connection with ladies' shoes.

The wood pulp layer is especially adapted 50 for use in a box toe or like stiffener for boots and shoes, as it is of light weight and inexpensive, and while it is preferred to incorporate this with the stiffening material above described, it is not desired to limit the invention in this respect, as good results may be 55 obtained when the wood pulp has incorporated with it other stiffening materials, such as tar, asphalt, gums and the like.

Claims:

- 60 1. A stiffening member for a boot or shoe comprising a wood pulp layer, a fabric layer and a stiffening composition comprising a soluble silicate and rubber latex applied to both layers and adhesively affixing said layers together.

2. A member for incorporation in a boot or shoe comprising a layer of wood pulp having applied thereto a composition of soluble silicate and latex.

3. A composite material adapted for use 70 as a stiffener comprising a supporting fabric, a mass of fibres derived from wood associated in a loosely-matted form with said supporting fabric, and, distributed throughout the interstices of said supporting fabric and said mass 75 of fibres, a continuous body of hardened saturant.

4. A composite material adapted for use as a stiffener comprising a foraminous supporting fabric, a mass of loosely-matted pulped 80 wood fibres supported by said foraminous fabric, and, distributed throughout the interstices of said foraminous fabric and said mass of loosely-matted pulped wood fibres, the residue of a dried saturant. 85

In testimony whereof, I have signed my name to this specification.

WALLACE C. BENNETT.